

Jan. 7, 1941.

C. PFANSTIEHL

2,228,235

HARDEDN BASE METAL PEN NIB

Filed March 28, 1940

Fig. 1.



Fig. 2.



Fig. 3.



Fig. 4.



Inventor:  
Carl Pfanstiehl.  
By Chittenden, Wiles, Davis, Mischel, Dawson.  
Atty's.

## UNITED STATES PATENT OFFICE

2,228,235

## HARDENED BASE METAL PEN NIB

Carl Pfanziehl, Highland Park, Ill., assignor to  
Pfanziehl Chemical Company, a corporation  
of Illinois

Application March 28, 1940, Serial No. 326,519

13 Claims. (Cl. 120—109)

This invention relates to a hardened base metal pen nib and a method of producing it, and more particularly to a ferrous metal pen nib upon which is integrally formed a hardened integral tip of altered chemical composition.

In my Patent 2,053,406, issued September 8, 1936, is described an integral steel pen nib and tip formed by the process therein described and more particularly described in my Patent 2,005,752, issued June 25, 1935. The pen nibs described in Patent 2,053,406, issued September 8, 1936, were preferably ferrous base materials, for example, steel. In my Patent 2,154,181, issued April 11, 1939, the use of a stainless steel pen nib of the austenitic 18—8 type is described. The pens described in these patents are considerable improvements upon pens of similar type theretofore known. However, they do not have the wear resistance of pen points formed in the usual way by welding a so called "Iridium" tip to a steel base. By means of the present invention, ferrous base integral nibs are hardened to produce a pen point which will have wear and corrosion resistance comparable with and, in many instances, actually better than those heretofore produced.

The invention is preferably carried out by adding to a base metal pen nib a hard, corrosion resistant base metal tip. Preferably the tip is produced in situ by alloying with the tip portion of the base a small amount of a hardening alloy.

The preferred hardening material is a mixture of chromium carbide and cobalt which has been assembled in the form of a minute pre-formed object, for example, in the form of a disc, cube or a rough sphere. This metallic hardening chemical, which itself is porous, soft, easily breakable and utterly unfit for pen point purposes, is preferably tacked to the pen nib, for example, as described in my Patent 2,005,752, or else by a light resistance weld, and then the integral nib is formed in the usual manner. The hardening chemical is thoroughly melted and absorbed by the steel base and no sharp line of division is indicated. On the contrary, the entire spheroid formed by the fusion is hardened by admixture with the hardening alloy material with it.

The alloy material may be prepared as desired, but the method hereinafter described for preparing it overcomes certain difficulties which are found in other methods of procedure.

As an example of the invention, chromium carbide was prepared by thoroughly mixing together

chromium and carbon in proportions to form Cr<sub>3</sub>C<sub>2</sub>.

This may be done, for example, by thoroughly mixing together about 86.7% by weight of pure electrolytic or other chromium powder of approximately 150 mesh and finer, with about 13.3% of powdered carbon, for example, obtained by grinding pure carbon or graphite rod or any other standard carbon material. The thoroughly mixed powders are placed in a small magnesium oxide crucible and heated in an electric furnace in a vacuum to about 2000° F. for 5 or 10 minutes. A pure reducing gas, preferably hydrogen, is then admitted to the furnace chamber at about atmospheric pressure and the temperature raised to 2700° F. and held there in the presence of the hydrogen for about an hour. In this process the materials combine to form Cr<sub>3</sub>C<sub>2</sub> which is removed from the furnace after cooling. The temperature used is low enough so that the material will readily pulverize. If the temperature is raised much above 2700° F., or if the heating is carried on too long, the mass begins to sinter and it is difficult to pulverize properly. Under the conditions the mass is only slightly sintered and can readily be ground in a mortar or ball mill to produce particles of 150 mesh or less.

The powdered chromium carbide so produced is then mixed with about 10% of cobaltic oxide (Co<sub>2</sub>O<sub>3</sub>) and 90% of chromium carbide, and covered with benzol or some other protective, inert, thin liquid and is ball milled for approximately 1½ hours. The mixed powders are then dried and again sifted through 150 mesh and pressed into minute granules in the shape of cubes or tiny flat discs, or any other convenient shape. This present operation should be carried out in a plastic die such as is described in my Patents 2,169,280 and 2,169,281, issued August 15, 1939. The amount of pressure employed is simply enough to hold the pressed material firmly in the desired shape. Usually 40 to 70 tons per square inch is sufficient, and in some cases lower pressures can be used. The pressed cubes or discs are then placed in a crucible—a large number may be placed in a single crucible—and heated to a bright red heat between 1500 and 1900° F. for a few minutes in hydrogen. The length of heating is such that the cubes will not stick together. In the treatment, the cobaltic oxide is reduced by the hydrogen to cobalt, which binds the small objects more strongly together. It also leaves them somewhat porous. The material, however, in this condition is utterly unfit for use as a pen

point. After forming, the granules are preferably tumbled to round off the edges somewhat. These hardening members are then lightly secured to the steel bases which are preferably of the 18-8 austenitic type stainless steel, either by condenser discharge tacking method described in Patent 2,005,752, or preferably by a light resistance weld. Preferably the amount of contact is kept at a minimum, as shown in the drawing, by tacking a corner of the granule to the nib. The blank with the hardening member so attached is then placed in a suitable apparatus for forming integral nibs, for example, as described in Patents 2,005,752 and 2,053,406. In this apparatus the hardening member and the nib are heated by an electric arc so that the hardening member and a portion of the steel are melted together to form a spheroidal tip. The chromium carbide disappears in the process, there being no clear line of division between the steel and any chromium carbide-cobalt alloy. Nevertheless, the tip of the pen is made extremely hard and completely corrosion resistant by this process. The tip formed resembles precisely an integrally formed tip. In composition it varies from about 80% or more of the chromium carbide alloy at the writing surface, to 40% or less at the part of the ball point nearest the body of the nib.

The product is illustrated diagrammatically in the drawing in which Fig. 1 represents a stainless steel pen blank 10 having a tip portion 11; Fig. 2 represents a perspective view of a small hardening cube 12; Fig. 3 is a view of the stainless steel pen nib blank 10 having the cube 12 lightly tacked to its tip 11; and Fig. 4 shows the pen blank 10 after the formation of the spheroid 13 by the fusion operation and after splitting the pen as indicated at 14.

The selection of a material for hardening presents some difficulties because hardening alloys tend to produce blow holes and do not produce generally dense close-grained hard tip structure, or have the necessary resistance to corrosion.

The cobaltic oxide is used in combination with the chromium carbide in preference to the use of pure cobalt, because for some reason the mixture of chromium carbide and cobaltic oxide presses far better and produces a better pre-formed hardening member than a mixture of chromium carbide and cobalt. The amount of cobaltic oxide should be between 5% and 20% of the chromium carbide. The hardening members are small in comparison to the size of the tip produced. For tips of ordinary size the hardening member in the form of a rough cube 0.025 inch on a side is satisfactory.

The invention may be practiced in a less satisfactory manner by pre-forming tipping granules of the chromium carbide-cobalt material in combination with a suitable amount of stainless steel. For example, a tip may be pre-formed in any suitable size by forming in any suitable manner a combination of the chromium carbide-cobalt alloy and stainless steel, the proportion of the stainless steel in the alloy being from 20% to 60%. This granule may then be welded to the pen nib in any satisfactory manner. The preferred form of the invention, however, is much more economical to practice, and furthermore provides a gradation of alloy within the tip which is not readily procurable in any other manner.

Instead of or in combination with the chromium carbide other refractory carbides compat-

ible with the metal of the pen nib may be employed. For example some of the chromium carbide may be replaced with molybdenum carbide or tungsten carbide or small amounts of it may be replaced with boron carbide.

Cobalt may be replaced in whole or in part by nickel or by iron. When using either of these metals, however, the tendency thereof to form carbides must be considered and if appreciable amounts of either are used it may be necessary to supply a slight excess of carbon to prevent the formation of an unsatisfied chromium carbide.

The foregoing detailed description has been given for clearness of understanding only, and no unnecessary limitations should be understood therefrom.

What I claim as new, and desire to secure by Letters Patent, is:

1. A stainless steel pen nib of the 18-8 type having integrally formed at the tip thereof a writing spheroid formed by fusion, said spheroid including a hardening metal not present in the body of the nib, said spheroidal writing surface being dense and close-grained. 25

2. The method of forming a pen point from ferrous metals comprising fusing the point of a ferrous pen nib while in contact with a granule of hardening metal, whereby an integral spheroidal writing surface embodying the material in the body of hardening metal is produced. 30

3. As a composition of matter, a formed minute body consisting essentially of a refractory steel compatible carbide and a binder of metal from the iron group. 35

4. As a composition of matter, a formed minute body consisting essentially of chromium carbide and a cobalt binder.

5. A composition as set forth in claim 4, in which the chromium carbide is essentially  $\text{Cr}_3\text{C}_2$  40 and the amount of cobalt is from 5% to 20% of the total.

6. A composition as set forth in claim 4, in which the chromium carbide is essentially  $\text{Cr}_3\text{C}_2$  45 and the amount of cobalt is approximately 10% of the total.

7. As a hardening member for pen nibs, a minute, pressed, slightly porous body containing approximately 80% to 95%  $\text{Cr}_3\text{C}_2$  and 5% to 20% Co, the Co having a distribution produced by reduction of a mixture of powdered  $\text{Cr}_3\text{C}_2$  and  $\text{Co}_2\text{O}_3$  in intimate pressed contact by heated hydrogen. 50

8. As a composition of matter, a formed minute body consisting essentially of an alloy of chromium carbide and cobalt, the chromium carbide being in the form of  $\text{Cr}_3\text{C}_2$  and representing from 80% to 95% of the total chromium carbide plus cobalt, together with an essentially ferrous metal, the ferrous metal representing from 20% to 60% of the total. 60

9. A pen nib having a body of austenitic 18-8 type stainless steel and having at the tip thereof a writing surface formed by fusion, said surface being substantially more corrosion resistant to ink than the body of the nib and consisting essentially of metal of the body of the nib alloyed with chromium carbide, the proportion of chromium carbide at the writing surface being in the order of 80% and diminishing rapidly away from the writing surface. 70

10. A stainless steel object comprising a body of austenitic 18-8 type stainless steel having integrally formed thereon by fusion of a portion of the body a minute tip containing a hardening 75

alloying metal consisting essentially of chromium carbide with a small amount of cobalt.

11. A stainless steel object comprising a body of austenitic 18-8 type stainless steel having integrally formed thereon by fusion of a portion of the body a minute tip containing a hardening alloying metal consisting essentially of a refractory steel compatible carbide containing a small amount of a cobaltic binder.
- 10 12. The method of forming a pen point from a metal pen nib comprising fusing the point of the pen nib while in contact with a granule of hardening metal the amount of hardening metal being so small, and it also being fused during 15 the process so completely, that the granule of hardening metal is completely disintegrated and distributed through the molten nib metal, and

freezing the molten metal into a small sphere, whereby an integral spheroidal writing surface embodying the material in the body of hardening metal is produced.

13. A pen including a metal nib having a tip integrally formed thereon by fusion of a portion of the nib, said integral tip having atomically distributed therein hardening metal, the concentration of hardening metal being greatest at the writing surface of the tip and diminishing rapidly 10 and steadily with distance therefrom, the tip being markedly harder and more corrosion resistant than the nib because of the presence of the atomically distributed material, there being no nucleus of the hardening metal and there being 15 nib metal at all parts of the tip.

CARL PFANSTIEHL.